

## UNITED STATES PATENT OFFICE.

BRODDE E. F. RHODIN, OF CALDWELL, NEW JERSEY.

## MAGNESIUM EXTRACTION.

No Drawing.

Application filed May 13, 1924. Serial No. 712,990.

*To all whom it may concern:*

Be it known that I, BRODDE E. F. RHODIN, a subject of the King of Great Britain, and a resident of Caldwell, county of Essex, 5 and State of New Jersey, have invented certain new and useful Improvements in Magnesium Extraction, of which the following is a specification.

This invention relates particularly to the 10 extraction of magnesium from magnesium alloys.

Under certain circumstances, for instance in the case of an over-supply of magnesium alloys, it may be that the magnesium content of the alloy may be of more value or more in demand than the alloy itself. The purpose of the invention therefore is to provide an inexpensive and practical method for effecting the separation of the magnesium from other elements with which it 20 has been combined.

The process has been found particularly practicable with the zinc, magnesium alloys and will therefore be described as applied 25 to such alloys.

Magnesium is one of the few metals that completely resists or is unaffected by the alkalis; metals as zinc, on the other hand, readily react with an alkali.

30 Briefly stated, the invention involves the subjection of the alloy to treatment in a molten alkali which causes the zinc or other metal in the treated alloy to react with the alkali and in the course of the same reaction the magnesium to separate itself from the other metal or metals and remain disassociated from the alkali.

Considering a practical illustration:

40 A bath of molten alkali, which may be either sodium hydroxide or potassium hydroxide is prepared in a kettle of cast iron or other suitable material and brought to a heat which need be only sufficient to initiate the reactions since the process becomes 45 exothermic and sufficient heat to complete the operations is supplied automatically as the reactions proceed.

The alloy may be supplied to the molten alkali either in the solid or in the molten 50 condition. In the reaction which takes place hydrogen is evolved and care should therefore be exercised that the feed of alloy be gradual and not excessive for the apparatus employed.

55 The zinc of the alloy being soluble in, the

alkali, reacts immediately with the alkali into zincate and hydrogen and the neutrality of the magnesium for the alkali results in the magnesium, in the presence of nascent hydrogen, separating in a practically pure state and floating to the top, where it can be readily removed.

As all magnesium produced by electrolytic decomposition has to undergo purification before being sold as a commercial product or before being used for alloying purposes, it may prove advantageous to add a small percentage of zinc to such crude magnesium and then proceed with the alkali purification process as above disclosed.

Magnesium in an extremely pure state can be produced by this process with very simple equipment.

What is claimed is:

1. The process of extracting magnesium 75 from magnesium alloys which comprises treating such alloys in a bath of molten alkali having chemical affinity for the metal or metals with which the magnesium is alloyed and for which the magnesium has 80 a natural chemical neutrality.

2. The process of extracting magnesium from magnesium containing alloys which comprises the preparation of a bath of molten alkali and the introduction into such 85 bath of the magnesium containing alloy in condition and quantity to control the exothermic action resulting from such combination.

3. The process of extracting magnesium 90 from magnesium-zinc alloys which comprises introducing such alloys at a regulated rate into a molten alkali bath of sodium or potassium hydroxide and mechanically removing the metallic magnesium released in 95 the ensuing reaction.

4. The process of extracting magnesium from magnesium containing alloys which comprises treating such alloys exothermically 100 with a molten alkali having a chemical affinity for the metal or metals other than the magnesium in the alloy and a natural chemical neutrality for the magnesium, thereby effecting complete separation of the magnesium and floatation of the same and thereafter removing said separated floated metal.

5. In the preparation of magnesium, the process which includes alloying with magnesium a metal having chemical affinity 110

for an alkali which has a natural chemical neutrality for magnesium and then treating the alloy of magnesium with such other metal in a bath of such molten alkali.

6. The process of extracting magnesium from magnesium alloys which comprises treating such alloys in a bath of molten alkali having chemical affinity for the metal or metals with which the magnesium is alloyed and for which the magnesium has a natural chemical neutrality and producing a combination of the alloying metal or metals with the alkali and a separation of

the magnesium in the presence of nascent hydrogen.

7. In the preparation of magnesium, the process which includes the addition of zinc to magnesium and the treatment in a bath of molten alkali to produce a combination of the zinc with the alkali and the separation of the magnesium in the presence of nascent hydrogen.

In witness whereof, I have hereunto set my hand this 28th day of March, 1924.

BRODDE E. F. RHODIN.